# EUROPEAN PATENT SPECIFICATION

(11) **EP 2 262 599 B1**
(45) Date of publication and mention of the grant of the patent: **12.11.2014**
(21) Application number: 09721920.8
(22) Date of filing: 20.03.2009
(51) Int. Cl.: B22F 5/10

(54) **NET-SHAPE OR NEAR NET-SHAPE POWDER ISOSTATIC PRESSING PROCESS**
ENDFORM- ODER ENDFORMNAHES ISOSTATISCHES PULVERPRESSVERFAHREN
PROCÉDÉ DE COMPRESSION ISOSTATIQUE DE POUDRE À FINITION IMMÉDIATE OU À FINITION PRESQUE IMMÉDIATE

(30) Priority: 20.03.2008 GB 0805242
(43) Date of publication of application: 22.12.2010
(73) Proprietor: Advanced Interactive Materials Science Limited, Edgbaston Birmingham B15 3BH (GB)
(72) Inventor: ARCHER, Geoffrey, Frederick, Lincolnshire PE9 4BA (GB)
(74) Representative: Barnes, Colin Lloyd
(86) International application number: PCT/GB2009/000757
(87) International publication number: WO 2009/115821

(56) References cited:
- EP-A- 0 815 995
- WO-A-97/40777
- WO-A-99/58273
- JP-A- 63 312 902
- M. H. BOCANEGRA-BERNAL: "Hot Isostatic Pressing (HIP) technology and its applications to metals and ceramics" JOURNAL OF MATERIALS SCIENCE, vol. 39, November 2004 (2004-11), pages 6399-6420, XP002532837

## Description

The invention relates to net-shape or near net-shape powder isostatic pressing processes, as applied to metallic and/or cermet/MMC (metal matrix composites) powder.

The invention is concerned particularly, but not exclusively, with the production of a bore of substantial length, typically longer than 750mm, in a component of hard wear-resistant material.

Such components can be made by Hot Isostatic Pressing (HIPing) but it is extremely difficult to produce bores in the formed components by machining. With difficulty, straight bores of small length such as 10mm can be machined. Prior art in relation to processes for Hot Isostatic Pressing includes US3992202, WO9411140, US2005/0214156, FR2796322 and EP1657010, but the prior art does not disclose method for the manufacture of net shaped components with helical bores using inserts which are subsequently removed.

We consider that it would be of advantage in certain circumstances to provide a bore of accurate dimensions extending lengthwise through a component of length approximately 2m, the component desirably being produced from a powder by a hot isostatic pressing process so as to provide hard wearing properties.

According to one aspect of the invention a method of producing a net or near net-shape component from metal powder comprises producing an insert of accurate dimensions corresponding to the dimensions of a bore to be created in the finished component, the bore having a length of at least 750mm, supporting the insert within a mould cavity, filling the mould cavity with metal powder, subjecting the powder to isostatic pressing, and subsequently removing the material of the insert.

As is well known, the mould may be an independent mould that is removed after an initial step to bind the powder together into a pre-form, and the pre-form is then encapsulated in a suitable containment which may be a canister or a sprayed coating, or a canister of suitable internal shape may be used as the mould, and the canister itself is evacuated prior to HIPing

Preferably the insert is supported in position in the mould cavity by a plurality of formers of a material that is compatible with the finally consolidated powder.

The insert may be a metallic insert of a material that is subsequently removable by chemical etching, preferably copper. The chemical etching may be assisted by electrolytic reaction.

In suitable cases the insert need only be coated with a material that can subsequently be removed by etching, in order to release the insert, which can then be extracted.

Preferably the metallic insert is coated with a suitable material that provides a diffusion barrier to prevent the material of the insert from diffusing by atomic diffusion into the powder being consolidated during HIPing.

The invention can enable a helical bore to be provided in a component.

Such a helical bore could be used for various purposes, such as to convey a fluid and/or to accommodate an electrical or fibre-optic cable to provide sensor or control system communications for example.

In one preferred embodiment a copper rod, of a diameter in the range of 6 to 10 mm for example and of length greater than 2m, is first bent into a helix of the required dimensions and this is then held in position in a powder containment prior to filling the containment with powder. The containment enclosing the powder, rod and former, is then consolidated by solid state diffusion using the HIPing method.

The diffusion barrier may be Al₂O₃ applied by vapour phase deposition or by high velocity spraying. Alternatively, the diffusion barrier may be created by applying boron nitride as an aqueous solution by spraying.

In a second embodiment a preformed metal tube, of 6mm to 10mm diameter for example, is filled with ceramic particles and is bent to a helical shape and placed within the powder containment prior to filling the containment with powder. The tube is held in position with formers compatible with the finally consolidated powder. The entire containment encompassing the metallic and/or cermet/MMC powder is then consolidated by solid state diffusion using the HIPing method.

During consolidation the metal tube may become totally diffusion bonded into the consolidated component but the ceramic particles will remain in the pre-process particle form and thereby can be removed mechanically via vibration techniques to leave a clean hole through the component.

### Example

The invention can be used to provide one or more holes in one or more helical lobes provided internally of the stator body of a helicoidal positive displacement pump, the stator body having a length of as much as 2m or more. Such stator bodies can be used to form the radially outer part of a linear motor and/or mud pump used in down-hole drilling. The hole or holes can be positioned to follow the core of a helical flute, which may have a pitch of about 1m and a radius of 50mm about the body axis. The helical lobes are defined by helical grooves in a mandrel that is positioned in the mould during pressing of the stator body.

## Claims

1. A method of producing a net or near net-shape component provided with a helical bore from metal powder comprising producing an insert of accurate dimensions corresponding to the dimensions of a helical bore to be created in the finished component, the bore having a length of at least 750mm, supporting the insert within a mould cavity, filling the mould cavity with metal powder, subjecting the powder to isostatic pressing, and subsequently removing the material of the insert, wherein the insert is a metallic insert of copper that is subsequently removable by chemical etching and the insert is coated with a material that provides a diffusion barrier to prevent the copper of the insert from diffusing by atomic diffusion into the powder being consolidated during HIPing.

2. The method of claim 1 in which the mould is an independent mould that is removed after an initial step to bind the powder together into a pre-form, and the pre-form is then encapsulated in a suitable containment.

3. The method of claim 2 in which the containment is a canister.

4. The method of claim 2 in which the containment is a sprayed coating.

5. The method of claim 1 or claim 2 in which the insert is supported in position in the mould cavity by a plurality of formers of a material that is compatible with the finally consolidated powder.

6. The method of claim 1. in which the chemical etching is assisted by electrolytic reaction.

7. The method of anyone of the preceding claims in which the insert is coated with a material that is amenable to removal by etching, and comprising the steps of releasing the insert by etching the coating, and then extracting the insert.

8. The method of claim 1 in which the diffusion barrier comprises Al₂O₃ applied by vapour phase deposition or high velocity spraying.

9. The method of claim 1 in which the diffusion barrier is created by applying boron nitride as an aqueous solution by spraying.

10. The method of claim 1 in which the insert is produced by taking a copper rod, of a diameter in the range of 6 to 10 mm and of length greater than 2m, bending the copper rod into a helix of the required dimensions, and then holding the helical rod in position in a powder containment prior to filling the containment with powder, the containment enclosing the powder, rod and former, and then consolidating the powder by solid state diffusion using a HIPing method.

11. The method of claim 1 in which the insert is produced by taking a preformed metal tube, of 6mm to 10mm diameter, filling the tube with ceramic particles, and bending the filled tube to a helical shape, placing the helical filled tube within the powder containment prior to filling the containment with powder, holding the tube in position with formers compatible with the finally consolidated powder, providing a containment encompassing the metallic and/or cermet/MMC powder, consolidating the contained material by solid state diffusion using a HIPing method and then removing the ceramic particles mechanically by a vibration technique to leave a clean hole through the finished component.

## Patentansprüche

1. Verfahren zum Produzieren einer endkonturgetreuen oder endkonturnahen Komponente, die mit einer schraubenförmigen Bohrung versehen wird, aus Metallpulver, das aus Folgendem besteht: Produzieren eines Einsatzes mit genauen Abmessungen, die den Abmessungen einer in der fertigen Komponente zu erzeugenden schraubenförmigen Bohrung entspricht, wobei die Bohrung eine Länge von mindestens 750 mm aufweist, Stützen des Einsatzes innerhalb einer Formkavität, Füllen der Formkavität mit Metallpulver, Unterwerfen des Pulvers einem isostatischen Pressen, und anschließend Entfernen des Materials des Einsatzes, wobei der Einsatz ein metallischer Einsatz aus Kupfer ist, das anschließend durch chemisches Ätzen entfernbar ist, und der Einsatz mit einem Material überzogen ist, dass eine Diffusionsbarriere bereitstellt, um zu verhindern, dass das Kupfer des Einsatzes durch atomare Diffusion in das Pulver, das während HiPing konsolidiert wird, diffundiert.

2. Verfahren gemäß Anspruch 1, bei dem die Form eine unabhängige Form ist, die nach dem anfänglichen Schritt entfernt wird, um das Pulver in einer Vorform zusammenzubinden, und die Vorform dann in eine geeignete Einfassung eingekapselt wird.

3. Verfahren gemäß Anspruch 2, bei dem die Einfassung ein Kanister ist.

4. Verfahren gemäß Anspruch 2, bei dem die Einfassung ein gespritzter Überzug ist.

5. Verfahren gemäß Anspruch 1 oder Anspruch 2, bei dem der Einsatz in der Formkavität durch eine Vielzahl von Formern eines Materials, das mit dem abschließend konsolidierten Pulver kompatibel ist, in Position gestützt wird.

6. Verfahren gemäß Anspruch 1, bei dem das chemische Ätzen durch elektrolytische Reaktion unterstützt wird.

7. Verfahren gemäß einem der vorhergehenden Ansprüche, bei dem der Einsatz mit einem Material überzogen wird, das der Entfernung durch Ätzen zugänglich ist, und das die Schritte des Lösens des Einsatzes durch Ätzen des Überzugs und dann des Extrahierens des Einsatzes beinhaltet.

8. Verfahren gemäß Anspruch 1, bei dem die Diffusionsbarriere Al₂O₃ beinhaltet, das durch Dampfphasenabscheidung oder Hochgeschwindigkeitsspritzen aufgebracht wird.

9. Verfahren gemäß Anspruch 1, bei dem die Diffusionsbarriere durch Aufbringen von Bornitrid als eine wässrige Lösung durch Spritzen erzeugt wird.

10. Verfahren gemäß Anspruch 1 bei dem der Einsatz produziert wird, indem eine Kupferstange, mit einem Durchmesser im Bereich 6 bis 10 mm und einer Länge größer als 2 m genommen wird, die Kupferstange in eine Schraubenform mit den erforderlichen Abmessungen gebogen wird, und dann die schraubenförmige Stange in einer Pulvereinfassung in Position gehalten wird, bevor die Einfassung mit Pulver gefüllt wird, die Einfassung das Pulver, die Stange und den Former einschließt, und dann das Pulver durch Feststoffdiffusion mittels eines HIPing-Verfahrens konsolidiert wird.

11. Verfahren gemäß Anspruch 1, bei dem der Einsatz produziert wird, indem ein vorgeformtes Metallrohr, mit 6 mm bis 10 mm Durchmesser, genommen wird, das Rohr mit keramischen Teilchen gefüllt wird, und dann das gefüllte Rohr auf eine schraubenförmige Form gebogen wird, das schraubenförmige gefüllte Rohr in der Pulvereinfassung platziert wird, bevor die Einfassung mit Pulver gefüllt wird, das Rohr mit Formern in Position gehalten wird, die mit dem abschließend konsolidierten Pulver kompatibel sind, eine Einfassung bereitgestellt wird, die das metallische und/oder Zement-/MMC-Pulver umschließt, das enthaltene Material durch Feststoffdiffusion mittels eines HIPing-Verfahrens konsolidiert wird und dann die keramischen Teilchen mechanisch durch eine Vibrationstechnik entfernt werden, um ein reines Loch durch die fertige Komponente zu hinterlassen.

## Revendications

1. Un procédé de production d'un composant à la forme ou presque à la forme muni d'un alésage hélicoïdal à partir d'une poudre métallique comprenant la production d'un insert aux dimensions exactes correspondant aux dimensions d'un alésage hélicoïdal à créer dans le composant fini, l'alésage possédant une longueur d'au moins 750 mm, le placement de l'insert à l'intérieur d'une cavité de moule, le remplissage de la cavité de moule avec une poudre métallique, la soumission de la poudre à une compression isostatique, et ensuite le retrait du matériau de l'insert, où l'insert est un insert métallique de cuivre qui est ensuite amovible par décapage chimique et l'insert est enduit avec un matériau qui offre une barrière de diffusion destinée à empêcher le cuivre de l'insert de se diffuser par diffusion atomique dans la poudre qui est consolidée au cours de l'opération de compression isostatique à chaud (HIP).

2. Le procédé selon la Revendication 1 dans lequel le moule est un moule indépendant qui est retiré après une opération initiale visant à lier ensemble la poudre en une préforme, et la préforme est ensuite encapsulée dans une enceinte adaptée.

3. Le procédé selon la Revendication 2 dans lequel l'enceinte est un bidon.

4. Le procédé selon la Revendication 2 dans lequel l'enceinte est un revêtement pulvérisé.

5. Le procédé selon la Revendication 1 ou 2 dans lequel l'insert est soutenu en position dans la cavité de moule par une pluralité de formeurs d'un matériau qui est compatible avec la poudre finalement consolidée.

6. Le procédé selon la Revendication 1 dans lequel le décapage chimique est assisté par une réaction électrolytique.

7. Le procédé selon l'une quelconque des Revendications précédentes dans lequel l'insert est enduit avec un matériau qui est apte à être retiré par décapage, et comprenant les opérations de libération de l'insert par décapage du revêtement, et ensuite l'extraction de l'insert.

8. Le procédé selon la Revendication 1 dans lequel la barrière de diffusion contient Al₂O₃, appliqué par dépôt en phase vapeur ou par pulvérisation haute vitesse.

9. Le procédé selon la Revendication 1 dans lequel la barrière de diffusion est créée par l'application de nitrure de bore sous la forme d'une solution aqueuse par pulvérisation.

10. Le procédé selon la Revendication 1 dans lequel l'insert est produit par la prise d'une tige en cuivre, d'un diamètre dans la plage de 6 à 10 mm et d'une longueur supérieur à 2 m, le pliage de la tige en cuivre en une hélice des dimensions requises, et ensuite le maintien de la tige hélicoïdale en position dans une enceinte à poudre avant le remplissage de l'enceinte avec de la poudre, l'enceinte contenant la poudre, la tige et le formeur, et ensuite la consolidation de la poudre par diffusion à l'état solide au moyen d'un procédé de compression isostatique à chaud (HIP).

11. Le procédé selon la Revendication 1 dans lequel l'insert est produit par la prise d'un tube métallique préformé, de 6 à 10 mm de diamètre, le remplissage du tube avec des particules de céramique, et le pliage du tube rempli en une forme hélicoïdale, le placement du tube hélicoïdal rempli à l'intérieur de l'enceinte à poudre avant le remplissage de l'enceinte avec de la poudre, le maintien du tube en position avec des formeurs compatibles avec la poudre finalement consolidée, la fourniture d'une enceinte englobant la poudre métallique et/ou de cermet/MMC, la consolidation du matériau contenu par diffusion à l'état solide au moyen d'un procédé de compression isostatique à chaud (HIP) et ensuite le retrait des particules de céramique mécaniquement par une technique vibratoire de façon à laisser un trou propre au travers du composant fini.
